

# United States Patent Office

2,860,945

Patented Nov. 18, 1958

1

2,860,945

## BLEACHING CYANOETHYLATED COTTON FIBERS WITH HYDROGEN PEROXIDE-PHOSPHATE SOLUTION AND OPTIONALLY WITH WATER-SOLUBLE SULFOXYLATE SOLUTION

Robert B. Dustman, Jr., Niagara Falls, N. Y., assignor to E. I. du Pont de Nemours and Company, Wilmington, Del., a corporation of Delaware

No Drawing. Application July 28, 1955  
Serial No. 525,064

10 Claims. (Cl. 8—110)

This invention relates to the bleaching of cyanoethylated cotton fibers and fabrics.

Cyanoethylated cotton is a relatively new type of fiber obtained by reacting cotton with acrylonitrile under alkaline conditions. The extent of cyanoethylation obtained varies with the conditions employed in carrying out the reaction. Fabrics containing cyanoethyl groups corresponding to from about 1.8 to 6.5% nitrogen have been reported. Presence of the cyanoethyl groups makes the modified cotton fiber resistant to micro-organism attack, more resistant than cotton to wet and dry heat degradation, more receptive to dyes, and more resistant to abrasion. (Parks, American Dyestuff Reporter, November 22, 1954, pages 774—779.) Although characterized by these desirable properties, which appear to be directly related to the presence of the cyanoethyl groups, these fibers have the distinct disadvantage of being difficult to bleach without causing serious reduction in their nitrogen content and consequent destruction of the desirable properties.

It is an object of the invention to provide an improved method for bleaching cyanoethylated cotton fibers and fabrics. A further object is to provide a method whereby such fibers can be successfully bleached without substantial reduction in their nitrogen content. Other objects will be apparent from the following description.

The objects of the invention are accomplished by subjecting cyanoethylated cotton fibers to the action of an aqueous alkaline solution of hydrogen peroxide whose alkalinity is due essentially to the presence of a molecularly dehydrated phosphate. In one embodiment of the invention, the fibers are also subjected to the action of an aqueous solution of a soluble formaldehyde sulfoxylate, preferably preceding the treatment with the peroxide solution.

It has now been found that cyanoethylated cotton fibers can be effectively bleached by the action of a hydrogen peroxide solution made alkaline by the presence of a molecularly dehydrated water-soluble phosphate without any significant reduction in the nitrogen content of the fibers resulting. The action of such a peroxide solution is rather unique in that peroxide solutions alkalized by means of caustic soda, sodium silicate or borax, all commonly employed in alkaline peroxide bleach formulas, cause excessive reduction of the nitrogen content of the fibers with consequent degradation of their desirable properties.

Greater fiber brightnesses than those obtainable by a peroxide treatment alone can be achieved by subjecting the fibers to a separate treatment with an aqueous solution of a soluble formaldehyde sulfoxylate. This separate treatment may follow or precede the peroxide treatment. If used, it is usually preferable that it precede the peroxide treatment. It has been found that such a treatment with a formaldehyde sulfoxylate is about twice as effective in increasing the brightness of the fibers as is sodium hydrosulfite, one of the most com-

2

mon bleaching agents of the reducing type. Furthermore, it bleaches without causing any significant reduction in the nitrogen content of the fibers.

The invention is illustrated by the following examples in which all percentages are percentages by weight.

### EXAMPLE 1

Samples of a sized greige cyanoethylated cotton fabric were treated with peroxide baths of various compositions to determine the bleaching effectiveness of the baths and their effect upon the nitrogen content of the fabric. The treatments involved immersing the sample in the bath for 1 hour at 180° F. (except as noted for Bath A) at a 40:1 weight ratio of liquor to fabric. The compositions of the baths evaluated are shown below. The treated samples were washed in water, air-dried and ironed, and their brightnesses (% reflectances) determined, using a Hunter multipurpose reflectometer. The nitrogen contents of the treated samples were determined by the Kjeldahl method. The results obtained are shown in the table.

#### Bath A

0.5% hydrogen peroxide ( $H_2O_2$ )  
0.24% borax  
0.24% of an alkyl aryl polyether alcohol, a wetting agent  
Bleaching was for 15 minutes at 195° F.

#### Bath B

0.3% hydrogen peroxide ( $H_2O_2$ )  
0.6% 42° Bé. sodium silicate (containing the equivalent of about 10%  $Na_2O$ , 25%  $SiO_2$  and 65% water)

#### Bath C

0.3% hydrogen peroxide ( $H_2O_2$ )  
0.24% tetrasodium pyrophosphate ( $Na_4P_2O_7$ )

#### Bath D

0.3% hydrogen peroxide ( $H_2O_2$ )  
0.24% of an alkyl aryl polyether alcohol, a wetting agent

#### Bath E

0.3% hydrogen peroxide ( $H_2O_2$ )  
0.35% borax  
0.24% magnesium sulfate ( $MgSO_4 \cdot 7H_2O$ )

#### Bath F

0.3% hydrogen peroxide ( $H_2O_2$ )  
0.6% 42° Bé. sodium silicate  
0.36% borax  
0.12% magnesium sulfate ( $MgSO_4 \cdot 7H_2O$ )

| Bath                   | pH   | Percent Reflectance | Percent Nitrogen |
|------------------------|------|---------------------|------------------|
| A.....                 | 8.5  | 49.8                | 2.86, 2.14       |
| B.....                 | 10.1 | 61.9                | 2.75, 2.72       |
| C.....                 | 9.4  | 62.7                | 3.13, 3.14       |
| D.....                 | 6.6  | 56.4                | 3.10, 3.13       |
| E.....                 | 8.7  | 54.4                | 3.13, 3.10       |
| F.....                 | 9.1  | 60.5                | 2.81, 2.90       |
| Greige, untreated..... |      | 34.2                | 3.19, 3.16       |

It will be noted from the table that of the 6 baths evaluated, only Bath C gave a final brightness (percent reflectance) above 57 without causing excessive reduction in the nitrogen content of the fabric.

### EXAMPLE 2

A sample of the greige fabric of the above example was subjected to a two-stage treatment. A 1% solution of normal zinc formaldehyde sulfoxylate was employed at a liquor to fabric ratio of 20:1 for 1 hour at

180° F. in the first stage. The fabric was then rinsed with water. The second stage involved a treatment for 1 hour at 180° F. at a liquor to fabric ratio of 40:1, employing a peroxide solution containing 0.6% hydrogen peroxide ( $H_2O_2$ ) and 0.24% tetrasodium pyrophosphate ( $Na_4P_2O_7$ ). The brightness (percent reflectance) after the second stage was 69.5%, while the final nitrogen content of the treated fabric was 3.18%, the same as for the untreated fabric.

The use of sodium formaldehyde sulfoxylate in place of the zinc compound produces similar results.

#### EXAMPLE 3

A sample of the sized, greige cyanoethylated cotton fabric of the above examples was immersed 0.5 hour at 180° F. in a 1% solution of normal zinc formaldehyde sulfoxylate at a liquor to fabric ratio of 40:1. The sample was rinsed in water then bleached employing a solution containing 0.6% hydrogen peroxide ( $H_2O_2$ ) and 0.24% sodium tripolyphosphate ( $Na_5P_3O_{10}$ ). Bleaching was continued for 1 hour at 180° F. at a liquor to cloth ratio of 40:1. The reflectance of the bleached sample was 71.0% and its nitrogen content was 3.12% compared with values of about 34.2% and 3.18%, respectively, for the untreated fabric.

#### EXAMPLE 4

A sample of the sized, greige, cyanoethylated cotton fabric of the above examples was bleached for 1 hour at 180° F. at a liquor to fabric ratio of 40:1 employing a bleach bath containing 0.3% hydrogen peroxide ( $H_2O_2$ ) and 0.24% tetrasodium pyrophosphate ( $Na_4P_2O_7$ ). The sample was rinsed in water and dried. The reflectance was 67.1%. The sample was then immersed for 1 hour at 180° F. in a 1% solution of normal zinc formaldehyde sulfoxylate using a 40:1 liquor to fabric ratio. After rinsing the sample in water and drying, its reflectance was 74.7% as compared with an original value of about 34.2%.

#### EXAMPLE 5

A sample of the above sized, greige, cyanoethylated cotton fabric was bleached 2 hours at 180° F. at a 40:1 liquor to fabric ratio employing a bath containing 0.6% hydrogen peroxide ( $H_2O_2$ ) and 0.24% sodium tripolyphosphate. The sample was then rinsed in water and dried. The reflectance was 72.0%. The sample was next immersed in a 1% solution of normal zinc formaldehyde sulfoxylate for 1 hour at 180° F. at a 40:1 liquor to fabric ratio. The sample was rinsed with water and dried and its reflectance was found to be 75.9% as compared with an original value of about 34.2%.

The agent employed for rendering alkaline the peroxide treating solution can be any water-soluble molecularly dehydrated phosphate, such as the alkali metal compounds of this class. Examples are the sodium pyrophosphates, sodium tripolyphosphate and sodium hexametaphosphate. Minor amounts of other conventional alkaline materials may be present but the alkalinity of the treating solution should be due essentially to a molecularly dehydrated phosphate, otherwise substantial decrease in the nitrogen content of the fiber results. Solutions entirely free of such other alkaline materials are preferred.

The sulfoxylate treating solution may contain as the active agent any water-soluble formaldehyde sulfoxylate, examples of which are sodium formaldehyde sulfoxylate, normal zinc formaldehyde sulfoxylate and basic zinc formaldehyde sulfoxylate.

The sulfoxylate and peroxide treatments may be applied in any desired sequence, although it is usually preferred that the peroxide treatment follow the sulfoxylate treatment. The treatments may be applied to fabric without first desizing the fabric, as illustrated in the 75

foregoing examples. However, the fabric can be first desized and then treated in accordance with the invention, in which case, a desizing treatment should be employed which will effectively desize without reducing the nitrogen content of the fabric. A 2% "Rapidase" enzyme solution applied for 1 hour at 180° F. at a liquor to fabric ratio of 20:1 is suitable for that purpose. "Rapidase," a textile desizing product of the Wallerstein Company, is a liquid enzyme preparation containing liquefying and proteolytic enzymes.

The concentration of soluble formaldehyde sulfoxylate in the sulfoxylate treating solution, if used, may be varied considerably depending upon the results desired. Concentrations of from about 0.5 to 5% are generally suitable, concentrations of from 1 to 3% being usually preferred. Such solutions can be used at any desired liquor to fabric ratio, e. g. from 40:1 to 1:1. Temperatures from room temperature to the boiling temperature are suitable, the lower temperatures requiring longer times than the higher temperatures. Preferred temperatures range from about 160 to 212° F.

The concentration of hydrogen peroxide ( $H_2O_2$ ) in the peroxide treating liquor will depend upon the amount of bleaching desired. Generally it will range from about 0.1 to 2% or higher, concentrations ranging from about 0.2 to about 1% (as  $H_2O_2$ ) being generally preferred. The content of molecularly dehydrated phosphate in the peroxide solution usually should be at least about 0.1% and may be as high as about 4% or somewhat higher, the preferred range being 0.5 to 3%. The conditions as regards temperature and liquor to fabric ratio indicated for the sulfoxylate treatment also apply to the peroxide treatment.

The method of the invention provides a way of increasing the brightness of cyanoethylated cotton fibers and fabrics without causing excessive reduction in their nitrogen contents. It, therefore, makes possible bleaching such materials without destroying or reducing those desirable properties of this type of fabric which are due to the presence of cyanoethyl substituent groups in the fiber.

I claim:

1. The method of bleaching cyanoethylated cotton fibers containing cyanoethyl groups equivalent to from 1.8 to 6.5% nitrogen based upon the weight of said fibers comprising bleaching said fibers with an aqueous alkaline solution of hydrogen peroxide in which the alkaline agent consists essentially of a water-soluble alkali metal molecularly dehydrated phosphate, at a temperature in the range from room temperature to the boiling temperature of said solution, said solution containing from 0.1 to 2%  $H_2O_2$  and from 0.1 to 4% of said phosphate.
2. The method of claim 1 carried out at a temperature within the range 160 to 212° F.
3. The method of claim 2 wherein bleaching is effected while the fibers are immersed in the hydrogen peroxide solution.
4. The method of bleaching cyanoethylated cotton fibers containing cyanoethyl groups equivalent to from 1.8 to 6.5% nitrogen based upon the weight of said fibers comprising bleaching said fibers in two separate bleaching treatments with solutions (1) and (2) at a temperature in each treatment between room temperature and the boiling temperature of the solution used, said solution (1) being an aqueous alkaline hydrogen peroxide solution in which the alkaline agent consists essentially of a water-soluble alkali metal molecularly dehydrated phosphate which is present at a concentration of from 0.1 to 4% along with from 0.1 to 2%  $H_2O_2$ , and said solution (2) being a 0.5 to 5% aqueous solution of a water-soluble sulfoxylate from the group consisting of the sodium and zinc formaldehyde sulfoxylates.
5. The method of claim 4 wherein the treatment with solution (1) precedes the treatment with solution (2).

6. The method of claim 4 wherein the treatment with solution (1) follows the treatment with solution (2).

7. The method of claim 4 wherein both treatments are carried out at a temperature within the range 160 to 212° F.

8. The method of claim 7 wherein the treatment with each solution is effected by immersing the fabric in the appropriate solution.

9. The method of claim 1 employing sodium pyrophosphate.

10. The method of claim 1 employing sodium tripolyphosphate.

References Cited in the file of this patent

UNITED STATES PATENTS

2,231,426 Kauffman ----- Feb. 11, 1941  
5 2,510,595 McEwen ----- June 6, 1950

OTHER REFERENCES

Chemical Abstrs. (1), 1940, 34, p. 8294<sup>1</sup>, abstract of J. Proc. Sydney Tech. Coll. Chem. Soc. 7, 61-64 (1935-37).

10 Chem. Abstrs. (2), 1944, 38, p. 2215<sup>2</sup>, abstract of Teintex 1941, 6, pp. 222-226.

Textile Colorist, pp. 407-411, September 1943.